

July 12, 1938.

A. B. GRAHAM

2,123,416

METHOD OF EXTRUDING METALS AND ALLOYS

Filed April 25, 1935

*Fig. 1.*



*Fig. 4*



*Fig. 5*



*Fig. 2.*



*Fig. 3.*



INVENTOR.

ALEXANDER BARBOUR GRAHAM,

BY  
Bynes, Stellens & Blenko

ATTORNEYS

## UNITED STATES PATENT OFFICE

2,123,416

## METHOD OF EXTRUDING METALS AND ALLOYS

Alexander Barbour Graham, Thornliebank, Glasgow, Scotland, assignor to The International Nickel Company, Inc., New York, N. Y., a corporation of Delaware

Application April 25, 1935, Serial No. 18,130  
In Great Britain May 1, 1934

2 Claims. (Cl. 207—10)

The present invention relates to a method of extruding metals and alloys, and more particularly to a method of producing articles, such as billets, rods, tubes, shapes or the like of metal or metal alloys by extrusion.

It is well known that heretofore, it has been the usual practice to cast a metal or alloy into an ingot which is to be extruded, and often to machine this ingot or a billet rolled therefrom until it fits the extrusion container. Certain shortcomings, limitations and disadvantages are inherent in the aforesaid process. Although attempts have been made to remedy the situation and to provide a more economical procedure, no proposal as far as I am aware has been wholly satisfactory and successful, particularly when conducted on an industrial scale for the manufacture of commercial acceptable products.

I have discovered that pieces or powder of metal or metal alloys if heated in a thin walled metallic container to a temperature below the melting temperature of such materials can be extruded directly from an extrusion press or chamber and that the initial materials will then coalesce so that billets, rods, tubes, shapes or the like can, in effect, be produced directly from initial materials which it has hitherto been thought necessary to melt and treat as described above prior to extruding.

It is an object of the invention to provide a simple, economical and practical procedure of extruding metals and alloys into various articles.

It is another object of the invention to provide relatively simple and compact apparatus for carrying the procedure into practice.

The invention also contemplates the provision of a practical procedure for producing articles like billets, rods, shapes, tubes or the like from metals and alloys by direct extrusion from pieces or powder of metals and alloys.

Other objects and advantages of the invention will become apparent from the following description taken in conjunction with the accompanying drawing in which:

Fig. 1 is a side elevation, partly in section and diagrammatic in character, of an embodiment of the novel apparatus for carrying the new process into practice;

Figs. 2 and 3 are views similar to Fig. 1 showing various stages of the process;

Fig. 4 is a modified embodiment of an apparatus to carry the present invention into practice; and

Fig. 5 is similar to Fig. 4 and shows the apparatus in another stage.

Broadly stated, the invention contemplates the heating in a thin walled metallic container of pieces or powder of a metal or of an alloy, preferably under the influence of a non-oxidizing atmosphere, especially a reducing atmosphere, to a temperature sufficiently high to effect subsequent coalescence of the pieces or powder under pressure but below the melting temperature of the metal or alloy. After heating the pieces or powder to such a temperature under the aforesaid condition, the heated pieces or powder and thin walled container are transferred to an extrusion chamber of an extrusion press while preventing the oxidation of the heated metal or alloy. In the extrusion press, pressure is applied to the heated pieces or powder preferably under the influence of a non-oxidizing atmosphere, especially a reducing atmosphere to such an extent that the heated pieces or powder of metal or alloy will coalesce and that billets, rods, tubes, shapes or the like can be extruded directly from the extrusion press or chamber. In this manner, the aforesaid articles can be produced directly from initial pieces or powder of a metal or an alloy which, heretofore it has been thought impossible and which heretofore it has been thought necessary to melt the pieces or powder and to cast the same into an ingot or billet which had to be rolled or worked to size in order to fit the extrusion chamber. In certain instances, it was even necessary to machine the ingot or billet. All of these prior operations have now been discovered to be unnecessary and the present invention provides the art with a simplified procedure.

The term "pieces" is intended to include shot, turnings, shavings and scrap of all kinds suitable for the production of billets and so forth.

In order to obtain complete homogeneity, the surfaces of the pieces or powder must be made clean initially and kept as clean as possible during the extrusion. If this is not done, that is to say if any oxide film or scale is left or allowed to form on the surfaces, it may be impossible to produce a coherent or usable article.

The invention is of particular value in the production of articles from metals or alloys that are normally difficult to extrude and particularly from pieces or powder consisting of or containing nickel.

The heating of the pieces or powder may, if desired, be effected in an auxiliary container and means may be provided for transferring the pieces or powder from this auxiliary container to the extrusion chamber without subjecting them to oxidation. Further, the auxiliary container may

be arranged either outside or inside the extrusion press. In the former case the auxiliary container may advantageously incorporate an electrical heating element and be arranged to move between a position in which it co-operates with a charging hopper or the like and a position in which it is in register with the extrusion chamber to discharge its contents. Again, the auxiliary container may communicate with the extrusion container or chamber by a pipe or its equivalent in which a non-oxidizing atmosphere is maintained and through which the heated pieces or powder are transferred to the extrusion container or chamber. If the heating is to take place in the press itself, the pieces or powder may be heated in the extrusion container or chamber electrically by means of high frequency induction, or similarly in an auxiliary container placed directly above the extrusion container or chamber and arranged so that, when heating of the contents is complete, these are allowed to drop into the extrusion container or chamber. The extrusion press-ram may either work through this heating container, or the heating container may be removed out of the way whilst extrusion takes place.

The powder or pieces may be heated in a thin walled container outside the extrusion press by any suitable means, for example, in a fuel-fired furnace or by a high frequency electrical method, this container then being transferred bodily with its contents to the press. The thin-walled container may then be extruded with the pieces or powder and either allowed to remain on the resultant extruded article as a cladding skin or removed by turning. Alternatively, the dimensions of the thin-walled container, the extrusion container or chamber and the press-ram may be so chosen that the thin-walled container acts in effect as a liner for the extrusion container or chamber.

The improved process may be carried into practice in any appropriate equipment but it is preferred to use the apparatus illustrated in the drawing.

Referring to the embodiment of the invention illustrated in Figs. 1 to 3, the powder or pieces of metal 1 are held in a thin walled metal container 2 which may completely enclose the powder or pieces or which may be open at the end, said container being placed in a block 3 which can slide on a table 4. This block 3 is formed with a central opening containing a liner 5 which is surrounded by an electric element serving to heat metal in the liner 5, for example, by high frequency induction. Appropriate means may be employed for maintaining a non-oxidizing atmosphere, especially one reducing in character, in the auxiliary chamber.

When the desired temperature has been reached, the whole block 3 is slid into position in the extrusion press by being pushed from the position shown in Fig. 1 to the position shown in Fig. 2, in which it lies above an extrusion container or chamber 7 and beneath a press ram 8. An extrusion opening 9 is provided at the bottom of the extrusion container or chamber 7. The pieces and thin walled container drop out of the block 3 into the extrusion container or chamber 7, which is then moved back into its initial position as shown in Figure 3, while the press ram 8 is then brought down so that the metal is extruded through the opening 9. As those skilled in the art will readily understand, appropriate means may be employed for maintaining a non-

oxidizing atmosphere, especially one reducing in character, in the extrusion chamber.

In the modified embodiment of the apparatus, shown in Figs. 4 and 5, the particles contained in a thin walled metallic container may be heated in any suitable furnace or by any suitable means, as those skilled in the art will readily understand instead of by the electrical heating unit shown in Figs. 1 to 3 before transferring to an extrusion press. The container 2 is transferred bodily with its contents 1 to an extrusion press as shown in Fig. 4. The heated container is then dropped into extrusion chamber 7 and press ram 8 is brought down to the position shown in Fig. 5 so that the metal is extruded through orifice opening 9. Appropriate means may be employed for maintaining a non-oxidizing atmosphere, especially one reducing in character, in the extrusion chamber as those skilled in the art will readily understand.

The apparatus illustrated in Fig. 1 may be modified by providing two or more extrusion chambers on one turntable arranged to rotate so as to bring each container in succession beneath the press ram, or again auxiliary heating containers may be provided in a turntable arranged to bring each in succession into register with the press ram and extrusion container or chamber. In either of these last two cases, the metal or metal alloy can be heated in one or more extrusion containers or chambers or auxiliary heating containers while extrusion is proceeding from another.

If grains of powder or very small pieces are used, they must be prevented from running out of the hole at the bottom or end of the extrusion container or chamber before extrusion begins, and accordingly the end of the container or chamber may be arranged to be closed mechanically, for instance, where an open ended thin walled container is used, or by a plug 10 or by a disc or similar piece of the metal or metal alloy to be extruded, forming, for example, the end wall of the thin walled metallic container. Moreover, if it is desired to compress the pieces or powder to some extent before extrusion proper begins, this closure will allow this to be done.

The invention may be applied not only to powder in which all the grains are free from one another, but to powder that has been sintered, for example, in a thin walled metal container, into the form of a block or blocks that will readily fit into the extrusion container or chamber. Such sintered blocks may be transferred hot to the extrusion press direct from the sintering chamber and converted into extruded solid articles in accordance with the invention, or they may be allowed to cool and be reheated prior to extrusion.

In the case of alloys, metal turnings or other scrap of the alloy in question may advantageously be used. However, the invention may also be applied to the production of alloys. In such a case, the ingredients from which the alloy is to be formed are placed in powdered form in a thin walled metal container in the extrusion press and in order to obtain the desired homogeneity the resultant extruded article may be annealed for a substantial time in order to allow the metals to diffuse into one another.

It will be understood that in every case the temperature of extrusion will depend on the metal or alloy in question and also on the form in which it is used, and that, while it must be sufficient to render the metal or alloy extrudable,

it must be below that at which the metal or alloy begins to melt. Thus in the case of nickel shot such, for example, as the pellets produced by the well-known Mond nickel carbonyl process, the temperature may be about 1150° C., while in the case of nickel powder, such, for example, as may be produced by the direct reduction of nickel oxide or salts, or by the decomposition of nickel carbonyl under conditions that prevent the formation of nickel shot, the temperature may be about 1220° C. Alloys of copper and nickel are preferably heated to a somewhat lower temperature, such as 1060° C., and "nickel-silver" alloys to a lower temperature still, such as 750° C. Nickel-iron powder, on the other hand, needs a higher temperature, such as 1200° C.

I claim:

1. A process of producing an article constituted of nickel or nickel alloy which comprises heating a mass of nickel containing particles in a thin-walled metallic container to a selected

temperature below the melting point of said mass and said container, transferring said container bodily to an extrusion chamber, and then extruding said heated container from an extrusion chamber whereby coalescence of the particles is effected and an integral nickel article is produced.

2. A process of producing an article constituted of nickel or nickel alloy which comprises electrically heating by means of high frequency induction nickel containing particles in a thin-walled metallic container to a temperature within a range of about 750° C. to about 1220° C., transferring said container bodily to an extrusion chamber through a reducing atmosphere, and then extruding said heated container from an extrusion chamber whereby coalescence of the particles is effected and an integral nickel article is produced.

20

ALEXANDER BARBOUR GRAHAM.